

## [54] COMBUSTIBLE COMPOSITIONS AND PROCESSES FOR THEIR PRODUCTION

[75] Inventor: Rodney T. Fox, North Humberside, England

[73] Assignee: Reckitt &amp; Colman Products Limited, England

[21] Appl. No.: 173,625

[22] Filed: Jul. 30, 1980

## [30] Foreign Application Priority Data

Aug. 2, 1979 [GB] United Kingdom ..... 26914/79

[51] Int. Cl.<sup>3</sup> ..... C10L 7/02; C10L 11/02[52] U.S. Cl. ..... 44/1 R; 44/7 D;  
44/16 R; 44/21[58] Field of Search ..... 44/16 R, 21, 25, 20,  
44/24, 41, 7 D, 1 R

[56]

## References Cited

## U.S. PATENT DOCUMENTS

|           |        |                     |         |
|-----------|--------|---------------------|---------|
| 3,338,691 | 8/1967 | Knowles et al. .... | 44/41 X |
| 4,083,697 | 4/1978 | Smith ....          | 44/24 X |
| 4,165,968 | 8/1979 | Duncan ....         | 44/41 X |

Primary Examiner—Carl F. Dees

Attorney, Agent, or Firm—Bacon &amp; Thomas

[57]

## ABSTRACT

An ignitable combustible composition comprising a matrix of solid resin having distributed therethrough combustible liquid, e.g. kerosene, water and contains also up to 25% by weight of expanded perlite to lengthen the burning time of a unit volume of the composition.

10 Claims, No Drawings

## COMBUSTIBLE COMPOSITIONS AND PROCESSES FOR THEIR PRODUCTION

## FIELD OF THE INVENTION

The present invention relates to combustible compositions and includes compositions which in relatively small size pieces are useful as firelighters and in larger pieces are suitable as firelogs, but which may be used as fuel.

## BACKGROUND OF THE INVENTION

A widely used type of firelighter is the so-called "white firelighter" first proposed by Shackleton inter alia in British Patent Specification No. 589594 and which is conventionally a block of hardened emulsion of aqueous curable resin and combustible liquid. The curable resin component forms on hardening a matrix containing water and the combustible liquid. Typically the combustible liquid is kerosene and the resin is an acid-cured urea formaldehyde resin. Compositions of this type are described in our British Patent Specification No. 1544635 and in British Patent Specification No. 1438944 which relate particularly to the inclusion of combustible particulate materials in firelighter compositions.

## PRIOR ART

French Pat. No. 1480979—Texaco Development Corporation discloses compositions for use as ignition products for fires or as heaters for such applications as dispelling frost from orchards. The compositions are wax or blends of waxes in solid form prepared by melting the wax(es) and floating on the surface of the molten wax a floatable material such as expanded perlite, vermiculite or glass microspheres to form a crust when the wax(es) has set solid and which acts to limit the area of surface from which volatiles may evaporate and combust during combustion of the wax(es) when the wax surface is liquified. These compositions are not match ignitable and need to be ignited by special means such as by pouring onto an exposed surface crust a quantity of a readily inflammable liquid such as a mixture of isooctane and kerosene which may be then ignited by means of, e.g. a candle.

"White firelighter" being a rigid structure, in which the rigidity is provided by the resin matrix, acts as a container for a liquid fuel in the form of the droplets of oil-in-water emulsion and is totally different from the abovementioned wax compositions in chemical constitution, method of making and especially physical structure which leads to a distinction in the mechanism of fuel burning. In the Prior Art proposals the composition is no more than a wickless candle with a broad base flame using the localised crust of floatable material as a wick replacement. In white firelighter compositions there is no wick and the fuel vapourises from an emulsion thereof to combust. White firelighter is prepared using emulsion technology and the emulsion is known to be sensitive to incorporation of particulates that have active sites on their surface where emulsion breakdown is initiated.

The incorporation of talc into white firelighter composition is known to lead to protraction of burning time for a standard block weight but there is no concomitant saving in kerosene utilisation. Furthermore, above a certain concentration addition of talc leads to breakdown of the firelighter emulsion prior to setting-up of

the resin which precludes the production of a rigid block.

## BRIEF DESCRIPTION OF THE INVENTION

5 We have now found that inclusion of expanded perlite in white firelighter produces protection in burning time per unit volume of composition with concomitant reduction in the volume of kerosene used.

10 Accordingly the present invention provides an ignitable combustible composition comprising a matrix of solid resin having distributed therethrough combustible liquid, water and up to 25% by weight of expanded perlite.

## 15 DETAILED DESCRIPTION OF THE INVENTION

The specific surface area of expanded perlite is 1 to 3 m<sup>2</sup>/g and depends to some extent on the degree of expansion of the perlite.

20 Preferably, the specific surface area of the expanded perlite is relatively small e.g. from 1 to 2 m<sup>2</sup>/g. The use of a further particulate material which may be one having a specific surface area exceeding 8 m<sup>2</sup>/g, e.g. at up to 1.2% by weight and preferably at about 0.6% by weight, e.g. 0.5 to 0.7% by weight of talc (specific surface area about 11 m/g) in addition to the expanded perlite is preferred. The use of significantly larger amounts than 0.6% by weight, e.g. greater than 1.2% by weight of talc or other materials having a high specific surface area tends to produce a soft composition, that is one that leaks kerosene, which may be useful in some respects but is not entirely suitable as a firelighter.

25 The combustible compositions may contain, in addition to the expanded perlite, a proportion of combustible particulate material, e.g. comminuted or granulated peat or wood as described in Specification No. 1544635; coal dust as described in Specification No. 1438944; seeds such as linseed, rapeseed and millet which may be used whole or crushed, or seed hulls such as coconut husk and peach stones are preferably comminuted; or mixtures thereof.

30 Specific surface areas may suitably be measured by the well-known gas adsorption method using nitrogen gas (B.E.T.) developed by Brunauer, Emmett and Teller.

35 The compositions of the invention may be prepared by mixing the expanded perlite and any other particulate materials with an aqueous emulsion of combustible liquid curable resin and emulsifying agent, adding a catalyst for the curing of the resin and allowing the mixture to set.

40 There is some danger of the addition of the particulate material particularly materials such as talc having a high specific surface area causing partial or total breakdown of the emulsion and the nature and amount of the material should be chosen to avoid this or to ensure that any emulsion breakdown is not excessive.

45 The amount of expanded perlite in the composition may be from 0.1 to 20% by weight but is preferably 1-3% by weight especially at least 1.5%.

50 Preferably, the combustible liquid is a hydrocarbon oil such as kerosene. Other combustible liquids which may be used include combustible oils of mineral origin such as white spirit and distillate, vegetable origin, such as corn oil, ground nut oil or animal origin such as fish oils and neatfoot oil. These may also be used in combination with kerosene. The combustible composition

may also contain combustible semi-solids such as waxes, e.g. slack wax and these may be dispersed or dissolved in the combustible liquid.

Whilst it is possible to operate the manufacture of white firelighter at slightly elevated temperatures, fire risk and other considerations then make the process hazardous. Therefore, the amount of solid wax or wax-like material that is incorporated into the combustible liquid preferably will not exceed a level beyond which the fluidity of the combustible liquid is impaired.

Roughly up to 60% by weight based on the combustible liquid present, of such wax or wax-like material may be incorporated. Preferably, from 20 to 50% w/w based on the weight of combustible liquid present.

The combustible liquid may comprise up to 93% w/w of the final combustible composition and is preferably, not more than 86% w/w of the final combustion. Valuable compositions can however be made using from 58 to 75% w/w of combustible liquid when care is given to selecting the expanded perlite and the amount of water in the composition.

The combustible composition may be produced in small pieces by moulding or a combination of moulding and cutting, these pieces being suitable for use as firelighters. Alternatively, the composition may be in larger pieces, or form a part of a composite larger structure intended for use as a fuel, for example in the shape of an artificial fire-log.

The compositions of the present invention are generally match ignitable although those compositions in which the water content is high are less easily so-ignitable. By adjustment of mixing technique whereby the water and expanded perlite are initially premixed, protracted burn time may be coupled with complete combustion and the match ignitability is enhanced.

The weight ratio of expanded perlite to water may be from 1:84 to 1:3, preferably 1:30 to 1:7.

In the case of a firelog, it is not necessary that all of the log be match ignitable, it is sufficient to provide a log which is largely non-match ignitable or difficult to light with a match but of which a portion is match ignitable and can act as a firelighter for the remainder. Such a log may be produced by moulding and setting a mixture as described above containing too much water to be match ignitable but having a desirably long burning time, and then moulding in a recess in the log a quantity of a composition according to this invention.

The present invention therefore includes a composite combustible composition comprising a non-match ignitable part having intimately attached thereto a match ignitable composition as described above.

The use of expanded perlite and any extra water used, may enable the amount of kerosene or other combustible liquid contained in a unit weight of composition to be decreased without the full expected decrease in burning time (proportional to the decrease in kerosene content), and may even extend the burning time despite the decrease in kerosene content.

Preferably, the composition contains from 14 to 20% by weight of water, more preferably about 20%. Generally, it is desirable to use as much water as possible without losing the capability of lighting the composition conveniently with a match.

The resin matrix may be urea-formaldehyde resin, a malamine-formaldehyde resin, a phenol-formaldehyde resin, or a phenol-furfuraldehyde resin. The most commonly used resin for making white firelighter compositions is an acid-cured urea-formaldehyde resin used as a

mixed precondensate dispersed or dissolved in aqueous medium optionally containing or to be used with extra urea or formaldehyde monomer and/or other known additives.

Broadly, any suitable thermosetting resin such as are discussed above may be used as is known in the art of white firelighter emulsion making. Crude phenols such as cresols may be employed provided a pure white product is not of importance.

10 Suitable catalysts for the particular resin system chosen are also well-known and are discussed in the published specifications referred to earlier.

The proportion of resin solids employed in the combustible compositions of the present invention is generally within the range 3% w/w to 8% w/w based on final composition.

If a large proportion of solids is employed then it may be desirable to use a relatively large resin content.

15 The combustible compositions of the present invention are typically produced by preparing an emulsion of combustible liquid in a resin dispersion using a suitable amount of suitable emulsifier. Such an emulsion may then be rapidly admixed with the desired amount of the expanded perlite and any other chosen particulate non-combustible or combustible solid, for example in a screw mixer. Catalyst may then be added and the mixture quickly poured into suitable moulds to gel. The moulds may be of size and shape to produce a small block for use as a firelighter without further processing. Alternatively, large blocks may be moulded for use as firelogs or still larger blocks may be made to be subsequently cut by knives or wires to produce blocks of a size suitable for firelighters or of a bigger size suitable for fuel.

20 35 If the expanded perlite is of large particle size it may prove difficult to cut blocks with wires whilst avoiding swarf, equally knives may be blunted rapidly and consequently such compositions are better moulded to the required size for use.

40 45 Selected solid combustible materials may be incorporated into the emulsion before, simultaneously with or after adding the expanded perlite. Suitable selected solid combustible materials include waste white firelighter optionally containing non-combustible granular waxes as part replacement for combustible liquid and the like.

It is thought that the use of the expanded perlite may improve the compositions by incorporating air into the composition.

Also the expanded perlite may act as a wicking agent improving the combustibility of the product and hence allowing more water to be used without losing the ability to light the composition by a match so that the extra water can extend the burning time.

The invention will be illustrated by the following Examples.

## EXAMPLES

60 65 The resin, emulsifier and catalyst and the method and order of mixing used in the following Examples was in each case the same save for Example 21. The resin used was a urea-formaldehyde resin dispersion in water containing 68% solids supplied by Ciba-Geigy as Resin Aerolite FL2 and the emulsifier is an emulsifying agent marketed by Lankro Chemicals Limited under the name Arylan SBC25. The catalyst was 1.3 N dilute hydrochloric acid used as a level of 0.5 parts dilute hydrochloric acid per 100 parts of final composition. In

Example 21 the urea-formaldehyde resin used was an aqueous dispersion supplied by Ciba-Geigy at 53% solids and identified as "XDF 4024," further the level of catalyst used was 0.6 parts per 100 parts of final composition. For convenience the acid has been included with the total water content in the table.

The appropriate amount of resin dispersion was diluted with water containing the emulsifier dissolved therein and the whole stirred whilst the kerosene was added to form an oil-in-water emulsion in known manner. An appropriate amount as indicated in the tables of expanded perlite and any other solid material was gently stirred into the emulsion. When the mixture was uniform catalyst was added with vigorous stirring and the block moulded immediately in a standard mould from which fingers of firelighter were cut by dividing the block into 12 equal parts.

-continued

| Particle Size<br>( $\mu$ ) | Particle Size Distribution<br>of Perlite (Grade 3JL) |  |
|----------------------------|------------------------------------------------------|--|
|                            | Concentration                                        |  |
| 125-500                    | 45.8%                                                |  |
| 75-125                     | 3.7%                                                 |  |
| 63-75                      | 0.93%                                                |  |
| 45-63                      | 0.93%                                                |  |
| 000-45                     | 0.00%                                                |  |

10

Expanded perlite of a specific surface area may be obtained from a grade with a given degree of expansion by a suitable choice of particle size. We have found on grading a sample of expanded perlite that particles of less than 63  $\mu$  have a specific surface area of about 1.6  $\text{m}^2/\text{g}$  and that particles retained by a BS16 sieve pro-

| Example No.                    | 1                 | 2                 | 3                              | 4               | 5               | 6               | 7     |
|--------------------------------|-------------------|-------------------|--------------------------------|-----------------|-----------------|-----------------|-------|
| Kerosene                       | %                 | 72.10             | 74.19                          | 70.88           | 78.88           | 75.88           | 73.61 |
| Total water (+Acid)            | %                 | 14.58             | 15.04                          | 14.38           | 14.36           | 14.36           | 19.63 |
| Resin solids                   | %                 | 4.04              | 4.16                           | 3.98            | 3.98            | 3.98            | 3.15  |
| Emulsifier solids              | %                 | 0.18              | 0.18                           | 0.18            | 0.18            | 0.18            | 0.18  |
| Talc                           | %                 | 0.61              | 0.63                           | 0.60            | 0.6             | 0.6             | 0.60  |
| Perlite                        | %                 | 8.50              | 5.80                           | 10.00           | 2.0             | 5.0             | 2.0   |
|                                | (Coarse<br>Grade) | (Medium<br>Grade) | (Fine<br>Grade)                | (EUP<br>100/21) | (EUP<br>100/21) | (EUP<br>100/21) | (3JL) |
| Finger weight (g)              |                   | 25.2              | 25.7                           | 32.7            | 34.6            | 23.6            | 31.6  |
| Burn time<br>(minutes-seconds) |                   | 15-32             | 14-45                          | 16-30           | 17-35           | 13-10           | 18-00 |
| <u>Burn time</u>               |                   |                   |                                |                 |                 |                 |       |
| Wt or Kerosene<br>in finger    |                   | 0.85              | 0.77                           | 0.71            | 10.64           | 0.74            | 0.87  |
| Example No.                    | 8                 | 9                 | 10                             | 11              | 12              | 13              | 14    |
| Kerosene                       | %                 | 66.11             | 59.11                          | 54.88           | 53.88           | 78.88           | 70.7  |
| Total water (+Acid)            | %                 | 25.82             | 31.76                          | 14.11           | 14.11           | 14.71           | 21.29 |
| Resin solids                   | %                 | 5.3               | 6.36                           | 4.24            | 4.24            | 3.64            | 5.83  |
| Emulsifier solids              | %                 | 0.18              | 0.18                           | 0.18            | 0.18            | 0.18            | 0.18  |
| Talc                           | %                 | 0.60              | 0.60                           | 0.60            | 0.6             | 0.60            | 0.60  |
| Perlite                        | %                 | 2.0               | 2.0                            | 1.0             | 2.0             | 2.0             | 2.0   |
|                                | (3JL)             | (3JL)             | (3JL)                          | (3JL)           | (<0.125mm)      | (3JL)           | (3JL) |
| Peat                           | %                 |                   |                                | 25.00           | 25.00           |                 |       |
| Finger weight (g)              |                   | 24.9              | 23.9                           | 40.8            | 35.80           | 32.9            | 24.7  |
| Burn time<br>(minutes-seconds) |                   | 31-40             | 33-50                          | 21-35           | 18-00           | 13-23           | 19-57 |
| <u>Burn time</u>               |                   |                   |                                |                 |                 |                 |       |
| Wt of Kerosene<br>in finger    |                   | 1.9               | 2.4                            | 0.96            | 0.93            | 0.52            | 1.1   |
|                                |                   |                   | difficult to<br>light by match |                 |                 |                 |       |
| Example No.                    | 15                | 16                | 17                             | 18              | 19              | 20              | 21    |
| Kerosene                       | %                 | 77.01             | 77                             | 77              | 77              | 78              | 71.67 |
| Total water (+Acid)            | %                 | 16.0              | 16                             | 16              | 16              | 16.2            | 12.96 |
| Resin solids                   | %                 | 4.24              | 4.2                            | 4.2             | 4.2             | 4.2             | 3.22  |
| Emulsifier solids              | %                 | 0.18              | 0.17                           | 0.17            | 0.17            | 0.17            | 0.15  |
| Talc                           | %                 | 0.6               | 0.6                            | 0.6             | 0.6             | 0.6             | —     |
| Perlite                        | %                 | 2.0               | 2                              | 2               | 2               | 1               | 11.94 |
|                                | (>BS16)           | (16-500 $\mu$ )   | (500-125 $\mu$ )               | (125-63 $\mu$ ) | (<63 $\mu$ )    |                 |       |
| Finger weight (g)              |                   | 28.8              | 34.7                           | 32.7            | 36.6            | 38.7            | 38.0  |
| Burn time<br>(minutes-seconds) |                   | 22-11             | 21-10                          | 20-50           | 18-05           | 21-25           | 21-10 |
| <u>Burn time</u>               |                   |                   |                                |                 |                 |                 |       |
| Wt of Kerosene<br>in finger    |                   | 1.00              | 0.79                           | 0.83            | 0.64            | 0.72            | 0.72  |
|                                |                   |                   |                                |                 |                 |                 |       |

| Particle Size Distribution<br>of Perlite (Grade 3JL) |               |
|------------------------------------------------------|---------------|
| Particle Size<br>( $\mu$ )                           | Concentration |
| >1000                                                | 6.5%          |
| 500-1000                                             | 42.1%         |

vided a specific surface area of 1.4  $\text{m}^2/\text{g}$  whereas intermediate size particles provided a higher specific surface area, e.g. 2 to 3  $\text{m}^2/\text{g}$ .

A "white firelighter" emulsion was prepared having the following composition.

|                                                                                 |  | % w/w |
|---------------------------------------------------------------------------------|--|-------|
| Urea + formaldehyde resin XDF 4024<br>(53% solids)                              |  | 6.94  |
| Emulsifier sodium dodecyl benzene<br>sulphonate (25% solids)<br>(ARYLAN SBC 25) |  | 0.70  |
| Water                                                                           |  | 10.45 |
| Kerosene                                                                        |  | 81.86 |
| Soap powder                                                                     |  | 0.05  |

To 700 g. portions of this emulsion were added in a first series increasing volumes of water only; and in a second series increasing volumes of water and 15 g. expanded perlite, EUP 100/28.

Each mixture was catalysed with 4.2 g. of 1.3 N hydrochloric acid and cast into a unit block which was cut into uniform pieces of the same volume, wrapped in PVC film, stored for 24 hour before conducting burning tests in quadruplicate on them. The results are tabulated below:

| Added water (ml)                   | 60           | 240         | 300          | 0           |              |             |             |
|------------------------------------|--------------|-------------|--------------|-------------|--------------|-------------|-------------|
| Perlite.                           | Pre-<br>sent | Ab-<br>sent | Pre-<br>sent | Ab-<br>sent | Pre-<br>sent | Ab-<br>sent | Ab-<br>sent |
| Average finger<br>wt. of block (g) | 43.31        | 41.03       | 43.50        | 47.65       | 34.88        | 40.70       | 40.98       |
| Average burn<br>time (min)         | 14.4         | 13.88       | 48.7         | 34.28       | 68.70        | 37.50       | 13.75       |
| Average burn time                  | .46          | .46         | 1.90         | 1.20        | 3.55         | 1.63        | .42         |
| Wt of Kerosene                     |              |             |              |             |              |             |             |

It can be appreciated from such results that the burn time of compositions in accordance with the present invention with a water content in excess of 30% overall show a surprising and marked protraction of burn time as compared with similar compositions lacking expanded perlite. At lower water concentrations there is little if any difference in increase of burn time although the addition of water and of expanded perlite results in a reduction in the overall kerosene concentration and it is surprising that the protraction in burn time in these cases is unaffected. It has to be observed that it becomes increasingly difficult to light the blocks with a match as the water content approaches 40%.

In the Examples, the burn time was measured by laying an oblong finger of composition on a grid or a tripod and lighting one corner with a match. The burn-

ing time taken was the total time from lighting to spontaneous extinguishing.

Firelighter blocks of the present invention have been found to be no less effective in lighting the bulk of housecoals to make fires on a hearth than are the best of previously known firelighters and in a majority of cases there is a distinct improvement in utilisation.

The present invention also includes a preferred composition in accordance with the invention, which is especially useful as a firelighter and, which comprises at least 5 parts of expanded perlite, from 5 to 25 part water, from 65 to 85 parts kerosene, and up to 1.2 parts of talc, parts being by weight.

I claim:

15. 1. An ignitable combustible composition comprising a matrix of solid resin having distributed therethrough combustible liquid, water and up to 25% by weight of expanded perlite.
20. 2. A combustible composition as claimed in claim 1, wherein the expanded perlite has a specific surface area of from 1 to 2 m<sup>2</sup>/g.
3. A combustible composition as claimed in claim 1, containing from 0.1 to 20% by weight of expanded perlite.
25. 4. A combustible composition as claimed in claim 1, containing from 10 to 20% by weight of water.
5. A combustible composition as claimed in claim 1 wherein the combustible liquid comprises kerosene.
30. 6. A combustible composition as claimed in claim 1, comprising a further particulate material having a specific surface area of more than 8 m<sup>2</sup>/g.
7. A combustible composition as claimed in claim 1, comprising a particulate combustible material.
35. 8. A process for producing a combustible composition as claimed in claim 1 which process comprises mixing the expanded perlite with an aqueous emulsion of combustible liquid, curable resin and emulsifying agent, adding a catalyst for the curing of the resin and allowing the mixture to set.
9. A composite combustible composition comprising a body of non-match ignitable combustible material having intimately attached thereto a portion of a match ignitable composition as claimed in claim 1.
40. 10. An ignitable composition as claimed in claim 1, which comprises at least 5 parts of expanded perlite, from 5 to 25 part water, from 65 to 85 parts kerosene, and up to 1.2 parts of talc, parts being by weight.

\* \* \* \* \*